

## UNITED STATES PATENT OFFICE

2,309,273

## MAKING DRYING OILS

Remmet Priester, Deventer, Netherlands; vested  
in the Alien Property CustodianNo Drawing. Application October 24, 1940, Serial  
No. 362,682. In the Netherlands January 6,  
1937

6 Claims. (Cl. 260—396)

The present invention relates to the manufacture of drying oils from glyceride oils having one or more hydroxyl groups in the fatty acid radical, castor oil being the best known representative of this group of oils.

Prior to the present invention, it was already known to convert those oils having one or more hydroxyl groups in the fatty acid radical into drying oils by splitting off water from the fatty acid radical.

It has been proposed to carry out the aforesaid process in two steps, by first liberating the fatty acid from the oil, converting this fatty acid by heating at a temperature of say 200° C. into an unsaturated acid with two double bonds in a conjugated neighbouring position and thereafter esterifying the acid thus obtained with a suitable alcohol.

For obvious reasons, a process which causes the splitting off of water from the hydroxyl groups of the hydroxy fatty acid radicals present in the castor or like oil, without causing liberation of any considerable amount of free acid from the glyceride oil, is advantageous. Such a reaction has heretofore been suggested, using sulphuric acid or certain other substances as the catalyst. Among the very satisfactory catalysts originally described in my earlier cases (including Ser. No. 181,467 filed Dec. 23, 1937, of which the present case is in major part a continuation and which has now matured into Patent 2,226,830,) may be mentioned pyrosulphate such as  $K_2S_2O_7$  potassium pyrosulphate.

Alkali metal pyrosulphate, such as the sodium and potassium, are very useful, and possess important advantages over many of the catalysts proposed in the prior art, particularly in that the said substances are solids that do not melt or liquefy during ordinary running of the process, they can accordingly be easily and readily and completely removed from the oil after the heating operation, they can be employed without causing undesirable darkening of the oil under treatment, they are cheap and can be produced easily and cheaply and from materials that are readily available everywhere (e. g. alkali metal bisulphate including miter-cake or alkali metal sulphate or many other commonly found alkali metal salts and sulphuric acid), and the drying oils produced may have a desirably low acid number.

For more completely describing the process, I give the following specific example, from Ser. No. 181,467:

## Example

First part.—Castor oil is stirred with 1% by weight of finely divided potassium pyrosulphate, and heated under vacuum whilst passing carbon dioxide through the liquid at a temperature from 180—240° C. for 4 hours. The temperature is slowly raised during the heating process until the distillation of water has ceased.

Second part.—The mixture may then be further heated for 3 hours at a temperature of 280° C. under the same working conditions in order to form a stand oil. After elimination of the catalyst in the usual way (e. g. by filtration or straining) a high grade drying oil product is obtained with valuable technical properties.

The product of the "first part" of the process (if filtered from the pyrosulphate) is a drying oil, light in color, of strong drying properties and with an acid number very little above that of the castor oil employed as starting material.

Instead of castor oil, other oils which are esters of hydroxy fatty acids can be treated by this process to produce drying oils, e. g. the triglyceride of dihydroxystearic acid.

It will be understood that a small percentage of the pyrosulphate is sufficient, e. g. from 0.1% to 5% may be employed, but preferably 0.2% to 1.5% is most satisfactory. Instead of the potassium salt, the sodium salt, or mixture of the sodium and potassium salts are also suitable.

The temperatures given in the example are suitable and satisfactory, but various temperatures in the first part of the process substantially over 150° C. and up to 260° C. may be used. In the second part of the process, temperatures over 260° C., up to 300° C., may be used. It is hardly necessary to state that the higher temperatures, especially if continued for a long time, may cause a higher acidity of the oil.

The time element given in the example is satisfactory. But, with somewhat higher temperatures, correspondingly shorter time periods can be used.

The carbon dioxide can be replaced by other inert gases, e. g. nitrogen, chimney gases (previously washed and dried, if desired), producer gas, coke oven gas, etc. Or if desired, the gas can be omitted, particularly if a vacuum be used.

The process produces a good yield of drying oil, and if care be used, to avoid discoloration of the oil, an oil is formed that is of good quality, and usable for all the common uses of drying oils.

As set forth in my copending case 181,468 filed

December 23, 1937 (now Patent 2,226,831), there may be a substantial rise in acid number in the oil, during the second part of the process, and this can be prevented by adding glycerol to the oil, before or during or after the first part of the process, and before the second part of the process. The amount of such glycerol may be about 1% or from 0.5 to 3%, more or less. Other not easily volatile active alcohols can be similarly used, e. g. sorbitol, cetyl alcohol, glycol, pentaerythritol. Or alkylene oxides such as ethylene oxide can be introduced into the oil, e. g. with the current of inert gas, during the second part of the process.

The drying oil produced by the present process has excellent drying properties, similar to those of Chinese tung oil, and shows a very fine light yellow color. With driers added, a film of the oil dries rapidly, to a strong film. A stand oil can be produced from these drying oils, e. g. as in the "second part" of the above example. The temperature for the formation may be 260-300° C., preferably 270 to 280° C.

I claim:

1. A process of making a drying oil which comprises heating a glyceride oil which is an ester of a hydroxy fatty acid, in the presence of a small amount of a pyrosulphate as a dehydrating catalyst, to a temperature substantially above 150° C., for a sufficient time to cause splitting off of water from the hydroxyl groups of the hydroxy fatty acid radical, and continuing the heating until substantial drying properties are developed in the oil, the pyrosulphate being one that is a solid and which remains solid throughout the process.

5 2. A process of making a drying oil which comprises heating castor oil with not more than a few percent of an alkali metal pyrosulphate, to over 150° C., until an oil having drying properties is produced.

3. A process of making a drying oil which comprises heating castor oil with not more than a few percent of an alkali metal pyrosulphate, to substantially over 150° C., while passing a 10 current of an inert gas through said oil, until an oil having drying properties is produced.

4. A process of making a drying oil which comprises heating castor oil with not more than a few percent of an alkali metal pyrosulphate, 15 to substantially over 150° C., while the oil is under a pressure substantially below atmospheric, until an oil having drying properties is produced.

5. A process of making a drying oil which 20 comprises heating castor oil mixed with not more than a few percent of pyrosulphate of an alkali metal, to about 180 to 240° C., for about 4 hours, while said oil is under vacuum and while passing a current of an inert gas through said oil.

25 6. A process of making a drying oil which comprises heating castor oil mixed with not more than a few percent of a pyrosulphate of an alkali metal, to about 180 to 240° C., for about 4 hours, while said oil is under vacuum and while passing a current of an inert gas through said oil, and 30 thereafter heating the said material to about 270 to 300° C., until thickening to stand oil consistency is effected.

REMMET PRIESTER.